

Sept. 8, 1925.

1,553,197

R. C. STANLEY  
METHOD OF SEPARATING NICKEL AND COPPER FROM  
COPPER NICKEL MATTES OR MATERIALS  
Filed Sept. 30, 1924



INVENTOR

Robert C. Stanley  
by his attorneys  
Byrnes, Stubbs & Farnam Co.

Patented Sept. 8, 1925.

1,553,197

# UNITED STATES PATENT OFFICE.

ROBERT C. STANLEY, OF STATEN ISLAND, NEW YORK, ASSIGNOR TO THE INTERNATIONAL NICKEL COMPANY, OF NEW YORK, N. Y., A CORPORATION OF NEW JERSEY.

## METHOD OF SEPARATING NICKEL AND COPPER FROM COPPER-NICKEL MATTES OR MATERIALS.

Application filed September 30, 1924. Serial No. 740,842.

To all whom it may concern:

Be it known that I, ROBERT C. STANLEY, a citizen of the United States, residing at Staten Island, Richmond County, New York, have invented a new and useful Improvement in Method of Separating Nickel and Copper from Copper-Nickel Mattes or Materials, of which the following is a full, clear, and exact description.

10 My invention relates to the separating of copper and nickel and the producing of commercial copper and commercial nickel from copper-nickel mattes or materials.

15 The drawing submitted herewith shows a preferred form of flow sheet employed in connection with my process.

In describing my process in its preferred form, I will consider it as starting with a nickel-copper matte obtained in any well known way from materials containing nickel and copper. These mattes, which are usually Bessemer mattes, contain varying proportions of copper and nickel; and the separation of their contained metals as commercial 20 nickel and copper, prior to my invention (described in United States Patent No. 1,351,877, dated September 7, 1920) was a long and expensive process involving a large 25 number of steps. The process of said patent greatly reduces the number of steps and the expense of the process.

30 My present invention is designed to still further reduce the number of steps and cheapen the process, while yet enabling me to recover the precious metals of the platinum group.

35 In carrying out my process in its preferred form, I smelt the copper-nickel matte in a cupola furnace with an alkali sulphide or a sulphide of an alkali metal, or a material which will produce an alkali sulphide. In practice, I prefer to use niter cake as a 40 relatively cheap material for this purpose, this being a crude bisulphate of soda.

45 The smelting furnace in which this operation is carried out is preferably provided with a forehearth for separating the slag from the molten sulphide. The molten sulphides run continuously from the forehearth 50 into large pots, where separation takes place. In these pots, the copper tops containing some nickel material, and the nickel bottoms containing some copper material, may be allowed to solidify; or after separation and

while the top is still molten, the top may be transferred in molten condition to the next operation.

During the period of settling and separation in these pots, nickel sulphide containing some copper sulphide, together with precious metals of the platinum group, will settle to the bottom, so that there will be two layers of sulphides in the pot. The upper layer consists of impure sulphides of sodium copper and iron, while the lower layer consists of impure nickel sulphide containing some sodium, copper and iron sulphides, and the various metals of the platinum group.

Whether the separation is in molten or solid form, the nickel bottoms are preferably charged into a second smelting cupola, where they are again smelted with an alkali sulphide or the sulphide of an alkali metal or a material which will produce an alkali sulphide. In this case, again, I prefer to use niter cake. The resulting molten sulphides are tapped into a vessel, where they are allowed to solidify, thus again separating the impure copper sulphide from the impure nickel sulphide, again producing a copper top and a nickel bottom. The smelting in this second cupola is preferably carried to such a point that the nickel bottom produced will contain not over 3% of copper, and preferably about 1%.

Instead of separation in pots as above described, I may take the molten sulphides from the forehearth of the first smelting furnace to a separating furnace, such, for example, as a reverberatory furnace, in which the sulphides are kept in a molten condition by heat supplied from the fuel of the furnace.

Two or more of these separating furnaces are preferably employed, for a group of matte-smelting cupolas, so that each separating furnace may be operated on the fill-and-empty method. That is, one separating furnace is supplied with its charge of molten sulphides from the smelting cupolas and this charge is allowed to settle, for example, during one shift of eight hours. While the separation into tops and bottoms is taking place in this furnace, another separating furnace is being charged with the molten sulphides for the same purpose.

These separating furnaces may be of any

desirable type, provided sufficient heat is supplied to keep the sulphides in molten condition and allow the separation thereof.

I also find that if these materials are held in the separating furnaces for some time, the sulphide of sodium will become oxidized and rise to the surface as sulphate of sodium, and may be removed and utilized in the smelting cupolas. In practice, I prefer to use this recovered soda in the second smelting operation.

During the period of settling and separating in the furnace, nickel sulphide containing some copper sulphide together with the precious metals of the platinum group will settle to the bottom, so that there will be two layers of sulphide in the furnace.

It will be understood that after either or both smelting operations, I may separate the impure copper sulphide from the impure nickel sulphide, either in molten condition or by allowing them to solidify. I may do away with the second smelting operation and take the first impure nickel bottoms in either solid or molten condition and subject them to the further steps which I will now describe.

The separated nickel bottoms from either the first smelting operation, usually containing about 6% of copper, or from the second smelting operation, containing not more than 3% of copper and separated in either molten or solid condition, are taken to a converter. For this purpose, the converter should be lined either with basic or neutral material. If the converter already contains a sufficient quantity of impure nickel sulphide in the molten condition, solid impure nickel bottoms may be added thereto, or the solid impure nickel bottoms may be pre-melted and this nickel material supplied to the converter.

In blowing this impure nickel material, the exothermic reaction with the air blown in is insufficient to maintain the temperature desired for the requisite reactions; consequently, I supply further heat units to the operation, preferably by mixing with the entering air a certain amount of combustible material, such as natural gas, oil, powdered coal, etc. The additional heat thus supplied is sufficient to cause a reaction between the nickel oxide and nickel sulphide to form metallic nickel.

In this operation, I prefer to reduce the sulphur to  $\frac{1}{2}$  of 1%, though the operation may be carried on in order to still further reduce the sulphur. For example, I may carry on the operation until the sulphur is reduced to substantially .01%, thereby producing commercial nickel containing a small percentage of copper.

In the preferred form of my process, I form the impure metallic nickel coming from the Bessemerizing operation into im-

pure nickel anodes. These impure nickel anodes, which preferably contain not over 3% of copper and also contain the precious metals of the platinum group, are then purified by an electrolytic process. In this process, the impure nickel is used as an anode from which the nickel is plated upon the cathode, which preferably consists of a sheet of pure nickel, the precious metals entering the slimes produced in the electrolytic cells from which they are recovered. The liquor of the cell is preferably continuously circulated through a cementing tank or tanks for removing the copper, the purified solution passing back to the cell. Iron may be removed from the solution, if desired, by any well known method.

Now, considering the copper tops, separated in either molten or solid condition from the sulphides of the smelting operations, these tops are taken directly to a converter or converters and blown in one operation to commercial blister copper.

This blowing or converting may be done in converters lined with basic, neutral or acid refractory material, but I preferably employ basic material for this lining, as by so doing the sodium sulphate produced by the oxidation of the sodium sulphide in the tops is recovered and may be used as flux in the separation furnace, thus effecting a further economy.

In practice, I prefer to thus treat the impure copper tops from the first smelting operation, but if I employ two smelting operations, I preferably take the impure copper tops from the second smelting operation, whether the method of hot or cold separation is employed, and charge them back into the first smelting operation. These copper tops serve the important function of enriching the copper content of the tops from the first smelting operation so that they may be blown direct into blister copper. They also serve to supply alkali sulphide for the first smelting operation, and in many cases will furnish a sufficient amount of this without fresh additions thereof in the first smelting. Copper revert may also be added to enrich the resulting sulphides in copper.

The advantages flowing from my present invention lie mainly in the great saving in the number of steps employed, and in the time, labor, metallic losses and overhead expense.

As above stated, while I prefer to employ two smelting operations, I may use only one such operation and other variations may be made in my process without departing from my invention.

I claim:

1. In the separation of nickel and copper from mattes and materials containing them, the steps consisting of partially separating

the copper material from the nickel material by furnace treatment, thereby producing nickel material containing a proportion of copper material and then blowing the said 5 nickel material directly into metallic nickel containing a small proportion of copper.

2. In the separation of nickel and copper from mattes and materials containing them, the steps consisting of smelting the matte 10 or material until nickel material is obtained by separation which contains not over about 6% of copper material, and then blowing said nickel material directly into nickel containing a small proportion of copper.

15 3. In the separation of nickel and copper from mattes and materials containing them, the steps consisting of smelting the matte or material, separating the product into copper tops and nickel bottoms, again smelting 20 the nickel bottoms, again separating the copper tops and nickel bottoms, and then blowing the nickel bottoms in molten condition directly into metallic nickel containing a small proportion of copper.

25 4. In the separation of nickel and copper from mattes and materials containing them, the steps consisting of smelting the matte or material, separating the product into copper tops and nickel bottoms, again smelting 30 the nickel bottoms, again separating the copper tops and nickel bottoms producing nickel material containing not over 3% of copper, and then blowing said nickel bottom material directly into metallic nickel containing 35 a small proportion of copper.

5. In the separation of nickel and copper from mattes and materials containing them, the steps consisting of partially separating the copper material from the nickel material 40 by furnace treatment, thereby producing nickel material containing a proportion of copper material, then blowing the said nickel material directly into metallic nickel containing a small proportion of copper, and 45 subjecting the metallic nickel thus produced to electrolytic refining.

6. In the separation of nickel and copper

from mattes and materials containing them, the steps consisting of smelting the matte or material, separating the product into 50 copper tops and nickel bottoms, again smelting the nickel bottoms, again separating the copper tops and nickel bottoms, then blowing the nickel bottoms in molten condition directly into metallic nickel containing a 55 small proportion of copper, and then subjecting the metallic nickel thus produced to electrolytic refining.

7. In the separation of nickel and copper from mattes and materials containing them, the steps consisting of partially separating the copper material from the nickel material by furnace treatment, thereby producing nickel material containing a proportion of copper material, then blowing the said 60 nickel material directly into metallic nickel containing a small proportion of copper, subjecting the metallic nickel thus produced to electrolytic refining, and recovering the 65 precious metals of the platinum group from 70 the slimes of the electrolytic process.

8. In the separation of nickel and copper from mattes and materials containing them, the steps consisting of partially separating the copper material by furnace treatment 75 and formation of copper tops and nickel bottoms, and then blowing said nickel bottom material directly into metallic nickel containing a small proportion of copper and blowing the copper tops into commercial 80 copper.

9. In the separation of nickel and copper from mattes and materials containing them, the steps consisting of smelting the matte or material, separating the product into 85 tops and bottoms to produce a nickel bottom containing not over about 6% of copper, and then blowing the nickel bottoms into commercial nickel containing a small proportion of copper and blowing the copper 90 tops into commercial copper.

In testimony whereof I have hereunto set my hand.

ROBERT C. STANLEY.